

## UNITED STATES PATENT OFFICE.

MILLER EUGENE CONRAD, OF ATLANTIC, IOWA, ASSIGNOR TO C. B. SCHOENMEHL INCORPORATED, OF WATERBURY, CONNECTICUT, A CORPORATION OF CONNECTICUT.

## VOLTAIC CELL.

No Drawing.

Application filed February 9, 1921. Serial No. 443,616.

*To all whom it may concern:*

Be it known that I, MILLER EUGENE CONRAD, a citizen of the United States, and resident of Atlantic, in the county of Cass and State of Iowa, have invented certain new and useful Improvements in Voltaic Cells, of which the following is a specification.

This invention relates to voltaic cells, and especially to an improved negative therefor.

10 Reference is called to specification forming part of Letters Patent granted to me February 3, 1903 No. 719,752, and my present invention is an improvement thereon as to the process therein described.

15 The above patent as well as some granted in the period intervening making use of sulphur, and especially the mechanical mixture of sulphur as a negative electrode, are open to several objections, such as increased 20 internal resistance and loss of rated E. M. F. because of ash.

An excess of sulphur whether in a chemical or mechanical compound makes and increases the internal resistance when used as 25 a negative element in a voltaic cell.

In the present invention an electrode or depolarizing element containing copper oxid or the other suitable metallic oxids mentioned in my former patent, is subjected to 30 the fumes or vapor of sulfur, and is impregnated with sulfur. This results in the

production of a depolarizing element with low resistance and developing relatively high voltage.

This process of impregnating the negative 35 element with the fumes or vapor of sulphur is especially practical when using oxid of copper, and is true whether the oxid is in powder, flaky scale, or in the form of a compressed and baked element, such as cylinders, rods or plates.

The fumes or vapor of sulphur may be introduced into the kiln or oven through a suitable apparatus from the outside, or the sulphur may be placed directly in the kiln 45 or oven. Either method is economical since the necessary heat for oxidizing the copper is greater than the heat necessary to fume or vaporize sulphur.

What I claim and desire to secure by 50 Letters Patent is,

1. A negative electrode for use in a voltaic cell comprising a body of a depolarizing oxid impregnated with the fumes of sulfur. 55

2. A negative electrode for use in a voltaic cell comprising a body of copper oxid impregnated with the fumes of sulfur.

Signed at Atlantic in the county of Cass and State of Iowa, this third day of February A. D., 1921. 60

MILLER EUGENE CONRAD.